

## UNITED STATES PATENT OFFICE

JEAN PAISSEAU, OF PARIS, FRANCE

PROCESS FOR THE OBTAINMENT OF SHEETS OF PLASTIC MATERIAL WHICH ARE  
COMBINED OR BACKED

No Drawing. Application filed May 25, 1928, Serial No. 280,648, and in France July 5, 1927.

In the current manufacture of plastic substances based upon nitro-cellulose or acetyl-cellulose, it is the usual practice to place together and unite two sheets, one of which is transparent and the other opaque, for the obtainment of novel effects.

For example, a thin sheet of artificial mother-of-pearl is backed by a sheet of opaque material, white or colored with black or various other pigments. The said opaque sheet is visible through the transparent material and forms a background. The device consisting of the two assembled sheets may be placed upon a strong and thick plate of a less expensive substance which serves as a support, and the whole may be used for the manufacture of solid objects.

However, this method offers certain disadvantages. The two thin sheets are caused to adhere together by the hot pressing process, after coating one or both sheets with a suitable solvent. Therefore to produce a successful operation, it is necessary to keep within the strict limits of temperature and pressure, since if the temperature becomes excessive, the substance will become softened and will sink down, thus changing its appearance, and if the temperature is too low, the adhesion is imperfect.

In this latter case, the two sheets will frequently separate during their handling in the manufacture of articles. This separation is almost inevitable when the thin sheets are softened by immersion in hot water, or in a suitable liquid, in order to mount them upon backing which cannot be spread out, such as a wood shoe heel.

The process according to the invention will obviate all such defects, and by the use of simple and effective means, I am enabled to produce backed sheets having all the advantages of the sheets obtained by the prior practice.

In principle, the said process is characterized by the coating in the cold state upon the sheet which is to be backed, of a fluid mixture, colored or not, which adheres to the sheet in an effective manner and may in certain cases form the backing itself.

The said coating substance comprises different constituents whose proportions must

be carefully calculated in order to obtain the desired effect.

For instance, if the operation is to be performed upon a sheet of artificial mother-of-pearl or like substance having cellulose acetate as a base, the mixture should comprise:

1. A certain quantity of acetyl-cellulose which gives a certain stiffness to the mixture and serves as binding material;

2. A suitable amount of a colored powder, or a metallic compound, or a lake colored by anilin dyes, or a white pigment and a solution of an anilin color, and in general, any suitable pigments;

3. A diluting liquid, which is sufficiently volatile to allow the rapid drying of the coating, and is so formed that in addition to the neutral substances serving exclusively as diluting bodies to afford the suitable consistency of the coating material for the purpose, it contains a solvent which is sufficiently active to attack the surface of the coated sheet in order to obtain the adhesion, the said solvent being however used in such quantity that it will not dissolve or buckle the said sheet.

A formula corresponding to the above indications is given as follows, solely by way of example:

|                             | Parts |
|-----------------------------|-------|
| Pigment                     | 7     |
| Ethyl lactate               | 25    |
| Methyl alcohol              | 50    |
| Ethyl acetate               | 25    |
| Cellulose acetate (plastic) | 7     |
|                             | 85    |

Obviously, each of the solvents or diluting liquids may be replaced by other products such as cyclohexanol, methyl acetate, acetone, methyl-ethyl-acetone, or the like, provided the mixture of such products forms a complex substance of a rather volatile nature and slightly attacking the plastic substance, but not appreciably softening it. For a coating upon a plastic substance having nitrocellulose as a base, instead of using cellulose acetate it is obviously preferable to use celluloid as a binding substance, as well as the proper liquids or solvents.

In practice the coating or point thus formed may be applied by any usual process,

either by the brush, the air-brush, or by a machine for varnishing, painting or sizing. Efforts will simply be made to apply a coat which is sufficiently thick and regular to form an opaque screen.

5 After the coating or layer has dried it has a flat or dull aspect which may be unfavorable when the backed sheet is to be used alone for the manufacture of fancy articles, such as lamp shades, or in general, all articles 10 made of thin material. In such cases it is an easy matter to give to the whole a sufficient polish whereby it will exactly resemble the product obtained by the adhesion of 15 two sheets as in the known methods. For this purpose I polish the coated sheet in the polishing press by the use of heat and pressure, according to the known polishing methods.

20 The aforesaid process has a further advantage from the fact that it offers multiple combinations which would be difficult to produce with the known methods.

In this manner I point by the stencil on the 25 reverse side of the sheet to be backed, variegated patterns which may be as varied as desired, by the combination of suitable colors, and can also shade off several tones to obtain shaded designs.

30 It will be easy to note the infinite diversity 35 of the hues which can be obtained by my said method. On the contrary, in the known methods of backing by the use of two pre-formed sheets, it is necessary to produce the colored sheets in large blocks which are then sliced, and this makes it very difficult and expensive to obtain sheets of widely varying hues, due to the enormous number of blocks which must be manufactured, and the difficulty of producing plastic blocks whose colors are the same throughout the several blocks.

40 I may further obtain novel aspects by applying successively two coats of paint having opposite tonality I obtain for instance a 45 dead appearance by first applying a bright color, optionally transparent, and then covering it, after drying, with a coat which is black or neutral, or dark, which thus forms a screen.

50 The aforesaid opaque black coat may contain lampblack, which is insoluble.

The sheet thus prepared is adapted for adhesion to a piece of thick plastic substance, as readily as the sheet obtained by the adhesion of two thin sheets by the known method. I obtain such adhesion in the usual manner, by coating the two sheets, thin and thick, with a suitable solvent, and by placing them in the press, using heat and pressure 60 for the proper time.

65 Due to my new method, the sheets are more closely united than by the current method in which the sheets must be perfectly dry. For this special use I may in fact cause the thin sheet to adhere to the thick sheet before the

coating on the first sheet has entirely lost its solvent.

70 By the same method, I am further enabled to obtain novel effects by crackling or by sets of lines. For this purpose I first coat a colored paint in which the amount of plastic material used as a binding is less than the amount of color. When drying, the layer, which lacks binding, will shrink and will form sets of cracks, these varying according to the relative amounts of color and of plastic material dissolved.

75 After this crackled coat has dried, I may readily use the same method to apply a layer 80 of black or dark paint, or one which has a favorable color, so as to form an opaque layer which appears in the interstices or cracks and thus affords a new artistic effect.

85 The said process is applicable not only to plastic substances of the artificial mother-of-pearl class, which are given by way of example as affording the most interesting results, but also to all other plastic material in thin sheets to which it is necessary, for any 90 reason, to give a backing forming a screen, or which are to be placed upon a thin sheet of a different color.

95 Also, according to the same principle, i. e. the use of a liquid consisting of a volatile mixture of such composition that it will only slightly attack the plastic substance I may 100 (1) either cause to adhere to one face of the latter a sheet of paper having a desired color, and herein the adhesion is obtained by placing the whole in the press with the use of heat and pressure, or (2) after the said paint or the like has been applied, I may cause to adhere to the coated face, by means of the same liquid, a sheet of spongy paper or a piece of thin cloth such as tarlatan, or wood in very thin sheets, or like strong and porous substances.

105 Such combinations afford a sheet of plastic material which due to the fact that it is rough 110 on one side will be adapted—as well as any veneering wood—for suitable adhesion to wood, for instance by a suitable carpenter's glue.

115 The tarlatan or like fabric is preferably substituted for paper, due to its greater strength, when it is desired to obtain a very substantial adhesion, as for instance for the production of thin bands of marquetry.

120 Due to this modification, the plastic substances can be used for cabinet making and for marquetry, and by a suitable combination of colors, a given substance will produce most widely varying effects.

125 For the use of my said new product in the boarding or box-making industry, I preferably employ a thin sheet of plastic material to the back of which is caused to adhere a sheet of paper of the proper color. These two pieces will adhere strongly together, and the 130

resulting product is used in the same manner as baryta paper.

By the use of the same principle, i. e., the use of a mixture as above described, I may further place upon one face of a sheet of plastic material which is sufficiently transparent and is optionally colored, a piece of fabric having a suitable decorative aspect. If the said fabric is woven of natural textile fibres, it will properly adhere due to the liquid employed, and it may then be incorporated into the sheet, so to speak, by placing in the polishing press the device consisting of the sheet backed by the fabric, adding if necessary a thin sheet of plastic material of the same kind, for protecting purposes.

As an interesting improvement, I may substitute for the said fabric of natural textile fibres, a fabric consisting of artificial silk. This latter is based preferably upon the use of nitro-cellulose if the fabric is to be applied to celluloid, or the use of acetate of cellulose if applied to a plastic substance containing acetyl-cellulose. For this special purpose, susceptible of widely varying decorative uses, the fabric may consist of a non-loaded artificial silk, for a most effective adhesion to the plastic substance.

I may further employ a colorless artificial fabric loaded with pearl essence. The fabric will sink into the plastic mass and thus becomes invisible, leaving in view only the pearl essence, which affords decorative effects (variable at will) due to its changing or opalescent hues.

Due to the said use of the artificial fabric which is caused to absorb the mixture according to the invention and will sink into the plastic mass to form a single body, I may thus provide a sheet of valuable use which can be cut or punched, milled, or otherwise treated, with as great facility as ordinary plastic material.

Claims:

1. Process for the manufacture of sheets of plastic material which are combined or backed, consisting in applying, on a sheet of plastic material, a layer of a mixture adapted to attack but superficially the said sheet of plastic material and composed of a plastic material similar to that of the said sheet dissolved in a volatile compound comprising a mixture of a solvent of the said material and of a volatile liquid unable to dissolve the said material.

2. Process for the manufacture of sheets of plastic material which are combined or backed, consisting in applying, on a sheet of plastic material, a layer of a mixture adapted to attack but superficially the said sheet of plastic material and composed of a plastic material similar to that of the said sheet dissolved in a volatile compound comprising a mixture of a solvent of the said material and of a volatile liquid unable to dissolve the said

material, and in subsequently subjecting said sheet thus prepared to the action of a polishing press.

3. Process for the manufacture of sheets of plastic material which are combined or backed, consisting in applying, on a sheet of plastic material, a layer of a mixture adapted to attack but superficially the said sheet of plastic material and composed of plastic material similar to that of the said sheet dissolved in a volatile compound comprising a mixture of a solvent of the said material and of a volatile liquid unable to dissolve the said material, a colored filling substance being added to the first named mixture.

4. Process for the manufacture of sheets of plastic material which are combined or backed, consisting in applying, on a sheet of plastic material, a layer of a mixture adapted to attack but superficially the said sheet of plastic material and composed of a plastic material similar to that of the said sheet dissolved in a volatile compound comprising a mixture of a solvent of the said material and of a volatile liquid unable to dissolve the said material, and in applying on said layer before drying a sheet of spongy and resistant material.

5. Process for the manufacture of sheets of plastic material which are combined or backed, consisting in applying, on a sheet of plastic material, a layer of a mixture adapted to attack but superficially the said sheet of plastic material and composed of a plastic material similar to that of the said sheet dissolved in a volatile compound comprising a mixture of a solvent of the said material and of a volatile liquid unable to dissolve the said material, and in applying on said layer before drying, a layer of fabric.

In testimony whereof I have hereunto affixed my signature.

JEAN PAISSEAU.

110

115

120

125

130